

## UNITED STATES PATENT OFFICE

WILLIAM H. ALLEN, OF DETROIT, MICHIGAN, ASSIGNOR, BY MESNE ASSIGNMENTS, TO  
PARKER RUST PROOF COMPANY, OF DETROIT, MICHIGAN, A CORPORATION OF  
MICHIGAN

## PROCESS FOR RUSTPROOFING ARTICLES OF IRON AND STEEL

No Drawing.

Application filed August 11, 1928. Serial No. 299,129.

The present invention relates to a process of "rust proofing" iron and steel.

Among the objects of the invention is to modify the known processes involving the use of phosphorus compounds so as to greatly shorten the time usually considered necessary for properly rust proofing the iron or steel articles.

Heretofore phosphoric acid and phosphates of some of the metals in acid solution have been used for the purpose of producing on iron or steel articles, a rust resisting coating and in such processes, it has been considered necessary to heat the solution containing the articles to boiling and to accurately control the conditions of the process, thereby utilizing considerable time in the treatment of a batch of the articles.

In the present process, the articles are merely dipped in the rust proofing solution and allowed to remain only a short period, whereupon they are removed and brought to a moderately high temperature and then cooled and washed. These steps of this process consume only a small fraction of the time required in the known processes.

The solution which I have found desirable for the present purpose is a dilute solution of ortho-phosphoric acid containing chromium phosphate. These solutions may be prepared in any suitable manner and should contain about 2½% phosphoric acid and about .175% of chromium combined as phosphate; these proportions are not fixed but may be varied to give good results, although the proportions mentioned are preferred.

Free phosphoric acid up to several percent more will not materially interfere with the results, while chromium in much larger amounts, even up to one per cent or more, will also give good results.

In using the solution, the articles are dipped cold or only moderately warm, as heating of the solution to any great degree will cause deterioration thereof. The solution may be used slightly warm but should not be allowed to heat to near its boiling point.

After the articles have been in the solu-

tion for a very short period, they are taken out and heated to a temperature of approximately 450° F., to convert the chromium phosphate into insoluble chromium pyrophosphate and after cooling, the articles are then subjected to a washing or brushing step to remove the loose powder of phosphate from the surface.

Iron or steel articles treated in the present process may be subjected to severe tests without indication of rust.

Now having described the invention and the preferred form of embodiment thereof, it is to be understood that the said invention is to be limited not to the specific details herein given but only by the scope of the claims which follow.

I claim:

1. The process of rust proofing iron or steel articles, which comprises dipping them into a solution containing chromium and phosphoric acid radical, and subsequently heating to a temperature sufficient to convert the chromium phosphate into chromium pyro-phosphate.

2. The process of rust proofing iron or steel articles, which comprises dipping them into a dilute solution containing chromium and phosphoric acid radical, and subsequently heating to about 450° F.

3. The process of rust proofing iron or steel articles, which comprises dipping them into a solution containing chromium phosphate and free phosphoric acid, then heating to about 450° F.

4. The process of rust proofing iron or steel articles, which comprises dipping them into a dilute solution containing chromium and phosphoric acid radical maintained well below the boiling point, and subsequently heating the articles to a temperature sufficient to convert the chromium phosphate into chromium pyro-phosphate.

5. The process of rust proofing iron or steel articles, which comprises dipping them into a solution containing chromium phosphate and free phosphoric acid maintained well below the boiling point, and subsequently heating the articles to a temperature suffi-

55

60

65

70

75

80

85

90

95

100

cient to convert the chromium phosphate into chromium pyro-phosphate.

6. The process of rust proofing iron or steel articles, which comprises dipping them into a solution containing about .175% chromium as chromium phosphate and about 2.5% free ortho-phosphoric acid at a temperature below the boiling point, then heating the said articles to about 450° F. and subsequently removing any loose powdery deposit therefrom.

WILLIAM H. ALLEN.

15

20

25

30

35

40

45

50

55

60

65